

July 19, 1955

G. T. HARRIS ET AL

2,713,537

COBALT BASE ALLOY

Filed Oct. 31, 1950



INVENTORS.  
GEOFFREY THOMAS HARRIS &  
HENRY CAVE CHILD

BY

Bussell and Harding

ATTORNEYS.

# United States Patent Office

2,713,537

Patented July 19, 1955

1

2,713,537

## COBALT BASE ALLOY

Geoffrey Thomas Harris and Henry Cave Child, Sheffield, England, assignors to William Jessop & Sons Limited, Sheffield, England, a British company

Application October 31, 1950, Serial No. 193,238

1 Claim. (Cl. 75—171)

This invention relates to cobalt base alloys and has for its object the provision of alloys from which castings may be made having good strength (particularly creep strength) and resistance to oxidation at elevated temperatures, for example, 750° C.

According to this invention alloys contain:

Carbon above 1% to 2.96%; silicon .35 to 1.07%; manganese .54 to 1.06%; nickel 7.8 to 12%; cobalt 35 to 57%; chromium 17.6% to 19%; boron 0 to 0.5%; and carbide-forming elements consisting of molybdenum 2.9% to 5.4%, vanadium 2.4% to 8.2%, and niobium 1.9% to 4.8%, and the remainder iron with unavoidable impurities.

Since tantalum is usually present with commercial niobium, the reference to niobium in this specification includes, besides the pure product, such amounts of tantalum as are usually present in commercial niobium, such, for example, as ferro-niobium.

Increasing the carbon within the range mentioned and using proportionately higher totals of the carbide forming elements (vanadium, molybdenum, niobium etc.) has the effects of increasing the creep strength but the cold ductility decreases. The amounts of carbon and carbide formers are therefore selected according to which of these properties is required to predominate or to the required degree of balance between the two.

For optimum results it is desirable to maintain a balance between carbon and the carbide formers, vanadium, tungsten, molybdenum, niobium, titanium and tantalum. For carbon of 1.01% the total of the carbide formers should be about 6.7% and for carbon of 3% the total of the carbide formers should be about 16%. Between the limits of carbon indicated proportionate quantities of carbide formers to those given should be employed.

The iron content is preferably as low as is consistent with economy and with the use of ferro-alloys for melting purposes. As an indication of preferred amounts of iron, a range of 10 to 20% may be mentioned.

Nickel is preferably kept low within the above range, but where castings from the alloys have to be machined it is then desirable to use a higher proportion of nickel within the above range not less than 10%.

The following are examples of alloys made according to this invention and in each example the balance consists of iron and the usual impurities:

2

In addition to having high creep strength the alloys according to this invention possess exceedingly high fatigue properties at elevated temperatures. For instance, alloy L. 457 has a fatigue strength of  $\pm 12$  tons/sq. in. at 850° C. for one hundred million cycles.

Where a cold ductility of the order of 1% is deemed satisfactory alloys with a specification of:

|    |                     | Per Cent |
|----|---------------------|----------|
| 10 | Carbon              | 2.2      |
|    | Manganese           | 0.8      |
|    | Silicon             | 0.5      |
|    | Nickel              | 10.5     |
|    | Cobalt              | 40.0     |
| 15 | Chromium            | 19.0     |
|    | Vanadium            | 5.6      |
|    | Molybdenum          | 4.0      |
|    | Niobium (+tantalum) | 2.8      |

20 are considered to be the most satisfactory. At 750° C. cast material of the above composition will sustain stresses of 22 tons/sq. in. and 17 tons/sq. in. for 100 and 1000 hours respectively, the minimum creep rate being  $2 \times 10^{-4}$  and  $1.5 \times 10^{-5}$  per hour respectively.

25 At 850° C. the material will sustain stresses of 12.5 tons/sq. in. and 8 tons/sq. in. for 100 and 1000 hours respectively, the minimum creep rates being  $2 \times 10^{-4}$  and  $1.2 \times 10^{-5}$  per hour respectively. The hot ductility of these castings is approximately 3%.

30 The illustrative drawing accompanying the specification shows a graph based on alloys made according to this invention and having as main constituents nickel about 10%, iron about 15%, chromium about 19% the balance being cobalt and usual amounts of silicon and manganese, plus the carbide formers vanadium, molybdenum and niobium in the ratio 1.4:1:0.7. The graphs were prepared on the mean of two tests on cold sand mould castings and the figures give the time to fracture in hours under a stress of 10 tons per square inch at a 40 temperature of 850° C. The shaded band represents alloys having particularly good properties.

Having thus described our invention, what we claim as new and desire to secure by Letters Patent is:

Metal alloys having high creep strength and consisting of carbon above 1% to 2.96%, silicon .35 to 1.07%, manganese .54 to 1.06%, nickel 7.8 to 12%, cobalt 35 to 57%, chromium 17.6 to 19%, boron 0 to 0.5%, and carbide-forming elements consisting of molybdenum 2.9 to 5.4%, vanadium 2.4 to 8.2% and niobium 1.9 to 4.8%, and the remainder iron with unavoidable impurities, the total percentage of elements in the carbide-forming group being between 6.7 and 16%; the proportion of the carbide-forming elements to carbon falling approximately within the shaded area on the drawing, that is, being substantially as follows: with carbon between 1 and 1.5% about 6.7 to 10% carbide formers; with carbon between 1.5 and 2% about 8 to 12% carbide formers; with carbon between 2 to 2.5% about 10 to

| Melt Reference | C    | Mn   | Si   | Ni    | Co   | Cr   | W     | Mo   | V    | Nb   | B     | Fracture time in hours with 10 tons/sq. in. at 850° C. | Minimum Creep Rate Per Hour | Type of Alloy |
|----------------|------|------|------|-------|------|------|-------|------|------|------|-------|--------------------------------------------------------|-----------------------------|---------------|
| L. 371-----    | 1.02 | 0.8  | 0.5  | 12    | 45   | 19   | ----- | 2.9  | 4.5  | 1.9  | ----- | 270                                                    | $1.5 \times 10^{-4}$        | As Cast.      |
| L. 457-----    | 2.38 | 1.0  | .82  | 11.0  | 40.5 | 18.3 | ----- | 2.9  | 5.8  | 2.9  | ----- | 481                                                    | $8 \times 10^{-5}$          | Do.           |
| L. 458-----    | 2.96 | 1.06 | 1.07 | 7.8   | 34.9 | 18.8 | ----- | 4.6  | 8.2  | 4.8  | ----- | 370                                                    | $7.2 \times 10^{-5}$        | Do.           |
| L. 459-----    | 1.01 | 0.8  | 0.5  | ----- | 57   | 19   | ----- | 3.0  | 4.7  | 2.1  | ----- | 471                                                    | $2.2 \times 10^{-5}$        | Do.           |
| L. 474-----    | 1.04 | 0.85 | 0.35 | 9.8   | 38.1 | 19.2 | 3.8   | 3.4  | 2.4  | 2.7  | 0.5   | 310                                                    | $1.4 \times 10^{-4}$        | Do.           |
| L. 513-----    | 2.21 | 0.94 | 0.84 | 9.7   | 37.8 | 17.6 | ----- | 3.4  | 5.2  | 2.0  | 0.5   | 140                                                    | $1.9 \times 10^{-4}$        | Do.           |
| L. 518-----    | 2.89 | 0.8  | 0.5  | 9.0   | 38   | 19   | ----- | 5.4  | 5.9  | 3.3  | ----- | 375                                                    | $4.9 \times 10^{-5}$        | Do.           |
| L. 629-----    | 1.07 | 0.92 | 0.66 | 9.9   | 40.2 | 17.8 | 3.01  | 3.26 | 2.96 | 3.05 | ----- | 256                                                    | $8.0 \times 10^{-5}$        | Do.           |
|                | 1.01 | .54  | .35  | 10    | 37.8 | 17.6 | ----- | 2.9  | 2.4  | 1.9  | ----- |                                                        |                             |               |

14% carbide formers; with carbon 2.5 to 3% about 12 to 16% carbide formers.

References Cited in the file of this patent

UNITED STATES PATENTS

2,030,343 Wissler ----- Feb. 11, 1936  
2,299,871 Baird ----- Oct. 27, 1942

2,309,372  
2,513,470  
2,537,477

Wissler ----- Jan. 26, 1943  
Franks ----- July 4, 1950  
Mohling ----- Jan. 9, 1951

FOREIGN PATENTS

Great Britain ----- Feb. 21, 1935